

1

3,408,179

**CORROSION-RESISTANT NICKEL-CHROMIUM ALLOYS WITH IMPROVED STRESS-RUPTURE CHARACTERISTICS**

Harry Lewis, Birmingham, and Ronald Alfred Smith, Stourbridge, England, assignors to The International Nickel Company, Inc., New York, N.Y., a corporation of Delaware

No Drawing. Filed Aug. 12, 1965, Ser. No. 479,323  
Claims priority, application Great Britain, Aug. 14, 1964,

33,351/64

2 Claims. (Cl. 75—171)

**ABSTRACT OF THE DISCLOSURE**

A corrosion-resistant nickel-chromium-base alloy of high chromium content (27% to 35%) possessing good stress-rupture properties at elevated temperatures and containing controlled amounts of titanium, aluminum, cobalt, molybdenum, carbon, boron and zirconium.

The present invention relates to nickel-chromium base alloys suitable for use under stress at elevated temperatures, and, more particularly, to high chromium, nickel alloys which manifest a combination of desired high temperature properties, including enhanced resistance to corrosive environments, such as the combustion products of impure fuel, and a satisfactory level of stress-rupture characteristics.

As is well known to those skilled in the art, nickel-chromium base alloys have found wide and diverse utilization in industry, particularly for high temperature applications wherein substantial resistance to stress-rupture is required. Such alloys as commercially employed typically contain the precipitation hardening elements titanium and aluminum, and chromium in an amount of about 15% to 20%, although a review of recent literature seemingly indicates a trend to using lesser amounts of chromium in certain nickel alloys to achieve a higher magnitude of stress-rupture characteristics. This accomplishment has usually been at the expense of resistance to corrosion.

In our British Patent No. 959,509, nickel alloys containing substantial amounts of chromium, to wit, 27% to 35%, are disclosed as having excellent resistance to corrosive environments. These alloys contained, in addition to chromium, about 1.5% to 2.5% titanium, about 0.5% to 1.1% aluminum, the combined amount of titanium plus aluminum being from 2% to 3.2%. It is also disclosed therein that while it might have been thought that higher amounts of titanium and aluminum would have resulted in a higher order of stress-rupture properties, the reverse was the case. In any event, these alloys manifested a stress-rupture life of the order of 50 to 140 hours when tested under a stress of 17 long tons per square inch (t.p.s.i.) at 750° C. in the wrought condition upon age hardening.

Now, notwithstanding the excellent resistance to corrosion afforded by the alloys described in the above-

2

mentioned British patent, for some purposes an improved level of stress-rupture properties is also required. It has now been discovered that marked improvement in the stress-rupture properties can be achieved without loss of corrosion resistance in such alloys through the incorporation of special amounts of both cobalt and molybdenum therein.

It is an object of the present invention to provide high chromium, nickel-base alloys which manifest excellent resistance to corrosive environments and which also exhibit a satisfactory level of high temperature stress-rupture properties.

Other objects and advantages will become apparent from the following description.

Generally speaking, the nickel-chromium base alloys of the present invention contain (by weight) about 27% to about 35% chromium, about 1.5% to about 2.5% titanium, about 0.5% to about 1.1% and preferably from 0.5% to 0.85% aluminum, the total titanium plus aluminum being from 2% to 3.2% and preferably from 2.2% to about 2.75%, from about 0.01% to 0.1% carbon, from about 0.001% to 0.01% boron, from about 0.01% to 0.1% zirconium, from 12% to 30% cobalt, from 1% to 7% molybdenum and the balance essentially nickel. The use of the expression "balance" or "balance essentially" in referring to the nickel content of the alloys, as will be understood by those skilled in the art, does not exclude the presence of other elements commonly present as incidental elements, e.g., deoxidizing and cleansing elements, and impurities normally associated therewith in small amounts which do not adversely affect the novel characteristics of the alloys. In this regard, silicon should not exceed about 1% and manganese and iron should not exceed 1% and 2%, respectively, the level of impurities otherwise being preferably kept as low as possible.

In carrying the invention into practice, the alloys can be prepared by conventional processing techniques well known to those skilled in the art, although vacuum melting is preferred. With regard to the heat treatment of the alloys, generally speaking, it comprises solution heating the alloys for about one to eight hours at a temperature within the range of 1050° C. to 1200° C., the alloys, upon cooling, being thereafter aged by heating for one to 24 hours within the temperature range of 600° C. to 800° C. A suitable heat treatment consists in solution heating for four hours at 1160° C. followed by air cooling and aging for 16 hours at 750° C. and again air cooling.

For the purpose of giving those skilled in the art a better appreciation and/or understanding of the invention, the following illustrative data are given:

A series of alloys were prepared in wrought form, the compositions being given in Table I. Alloys Nos. 1 through 5 are outside the scope of the invention, Alloy No. 6 being within the invention. Each of the alloys was tested for stress-rupture characteristics by subjecting wrought specimens to a stress of 17 t.p.s.i. at 750° C., the alloys having been solution heated for four hours at 1160° C., air cooled, aged for sixteen hours at 700° C. and again air cooled. The life-to-rupture in hours and tensile elongation in per cent are also given in Table I:

TABLE I

| Alloy No. | Composition (percent by weight) |      |      |      |       |      |      |      |      |       | Stress, Rupture Properties at 17 t.s.i./750° C. |               |
|-----------|---------------------------------|------|------|------|-------|------|------|------|------|-------|-------------------------------------------------|---------------|
|           | C                               | Cr   | Ti   | Al   | Ti+Al | Co   | Mo   | Si   | Zr   | B     | Hours                                           | El. (percent) |
| 1         | 0.04                            | 30   | 1.7  | 0.8  | 2.5   | —    | —    | <0.2 | 0.05 | 0.003 | 135                                             | 2.2           |
| 2         | 0.06                            | 30   | 1.7  | 0.8  | 2.5   | —    | —    | <0.2 | 0.05 | 0.003 | 125                                             | 4.2           |
| 3         | 0.04                            | 30.4 | 1.52 | 0.81 | 2.33  | 19.1 | —    | <0.3 | 0.06 | 0.001 | 135                                             | 1.9           |
| 4         | 0.05                            | 30   | 2.0  | 1.0  | 3.0   | —    | 4    | 0.5  | 0.05 | 0.003 | 139                                             | 7.8           |
| 5         | 0.06                            | 30   | 1.7  | 0.8  | 2.5   | —    | 4    | 0.5  | 0.05 | 0.003 | 93                                              | 6.7           |
| 6         | 0.068                           | 31.0 | 1.90 | 0.55 | 2.45  | 18.0 | 4.68 | <0.3 | 0.06 | 0.004 | 365                                             | 6.6           |

The data of Table I clearly illustrate the beneficial effect in stress-rupture properties achieved with the co-presence of cobalt and molybdenum. Alloy No. 3 which contained about 19% cobalt but which was molybdenum-free did not afford any appreciable increase in stress-rupture life over those alloys devoid of cobalt. The same is true with regard to the cobalt-free but molybdenum containing Alloys Nos. 4 and 5. However, the co-presence of molybdenum and cobalt resulted in the marked increase of stress-rupture life, the increase being well over 150% of the stress-rupture lives of Alloys Nos. 1 and 2.

our British Patent No. 959,509, that the contents of titanium and aluminum, both individually and combined, be within the ranges specified herein, since departure therefrom, at least in any appreciable degree, leads to a marked fall in the stress-rupture properties. This is clearly shown by the results in Table III which relate to alloys heat treated and tested in the same manner as the alloys of Tables I and II. Alloys Nos. 6, 11, 15 and 15 in this table are in accordance with the invention, the others are not.

TABLE III

| Alloy No. | Composition <sup>1</sup> (percent by weight) |      |      |      |       |      |      |      |       | Stress, Rupture Properties at 17 t.s.i./750° C. |               |
|-----------|----------------------------------------------|------|------|------|-------|------|------|------|-------|-------------------------------------------------|---------------|
|           | C                                            | Cr   | Ti   | Al   | Ti+Al | Co   | Mo   | Zr   | B     | Hours                                           | El. (percent) |
| 13        | 0.043                                        | 29.4 | 1.43 | 0.56 | 1.99  | 19.7 | 3.98 | 0.05 | 0.003 | 135                                             | 6.0           |
| 6         | 0.068                                        | 31.0 | 1.90 | 0.55 | 2.45  | 18.0 | 4.68 | 0.06 | 0.004 | 365                                             | 6.6           |
| 11        | 0.038                                        | 30.6 | 1.72 | 0.82 | 2.54  | 19.2 | 4.00 | 0.07 | 0.001 | 351                                             | 3.0           |
| 14        | 0.027                                        | 30.8 | 1.73 | 0.84 | 2.57  | 19.3 | 3.99 | 0.07 | 0.002 | 294                                             | 4.2           |
| 15        | 0.09                                         | 30.9 | 2.14 | 0.65 | 2.79  | 18.0 | 4.48 | 0.06 | 0.003 | 263                                             | 4.5           |
| 16        | 0.058                                        | 30.4 | 2.41 | 1.13 | 3.54  | 19.2 | 3.80 | 0.07 | 0.002 | 170                                             | 3.8           |
| 17        | 0.018                                        | 30.4 | 2.39 | 1.15 | 3.54  | 19.2 | 3.99 | 0.07 | 0.002 | 133                                             | 2.2           |

<sup>1</sup> Alloys contained less than 0.3% silicon.

The effects of varying cobalt and molybdenum are shown by the results in Table II, the alloys therein having been treated and tested as described above in connection with the alloys of Table I. Alloys Nos. 6 and 8 to 11, inclusive, are in accordance with the invention, whereas the other alloys are not but which are shown for purposes of comparison.

As referred to above herein, the alloys of the invention are possessed of good resistance to corrosive environments, including, for example, the combustion products of impure fuel. In this connection and as indicated in our British Patent No. 959,509, it is considered that the corrosive attack brought about by the combustion products of such fuels is attributable to sulfates and chlorides in

TABLE II

| Alloy No. | Composition (percent by weight) |      |      |      |       |      |       |      |       | Stress, Rupture Properties at 17 t.s.i./750° C. |       |               |
|-----------|---------------------------------|------|------|------|-------|------|-------|------|-------|-------------------------------------------------|-------|---------------|
|           | C                               | Cr   | Ti   | Al   | Ti+Al | Co   | Mo    | Si   | Zr    | B                                               | Hours | El. (percent) |
| 4         | 0.06                            | 30   | 2.0  | 1.0  | 3.0   | 4    | 0.5   | 0.05 | 0.003 | 139                                             | 7.8   |               |
| 7         | 0.07                            | 30.6 | 2.27 | 0.65 | 2.92  | 8.9  | 4.07  | <0.3 | 0.06  | 0.003                                           | 179   | 3.4           |
| 8         | 0.09                            | 31.0 | 2.05 | 0.65 | 2.70  | 13.2 | 4.68  | <0.3 | 0.06  | 0.003                                           | 208   | 6.6           |
| 9         | 0.10                            | 31.2 | 2.03 | 0.65 | 2.68  | 21.7 | 4.79  | <0.3 | 0.06  | 0.003                                           | 296   | 7.0           |
| 10        | 0.09                            | 31.3 | 1.99 | 0.55 | 2.64  | 27.1 | 4.75  | <0.3 | 0.08  | 0.004                                           | 343   | 9.5           |
| 3         | 0.04                            | 30.4 | 1.52 | 0.81 | 2.33  | 19.1 | ----- | <0.3 | 0.08  | 0.001                                           | 135   | 1.9           |
| 11        | 0.038                           | 30.6 | 1.72 | 0.82 | 2.54  | 19.2 | 4     | <0.3 | 0.07  | 0.001                                           | 351   | 3.0           |
| 6         | 0.068                           | 31.0 | 1.90 | 0.55 | 2.45  | 18.0 | 4.68  | <0.3 | 0.06  | 0.004                                           | 365   | 6.6           |
| 12        | 0.096                           | 28.8 | 1.86 | 0.90 | 2.78  | 17.7 | 7.58  | <0.3 | 0.07  | 0.004                                           | 154   | 8.6           |

It will be seen from Table II that with cobalt and molybdenum contents in the ranges 12% to 30% and 1% to 7%, respectively, lives of at least 200 hours are generally obtained under the heat treatment and test conditions used. In consistently obtaining an optimum combination of high stress-rupture life and good ductility, together with maximum resistance to corrosion, it is advantageous that the alloys contain about 27% to 35% chromium, about 1.5%, and preferably 1.6%, to 2% titanium, about 0.5% to 0.85% aluminum, the total titanium plus aluminum being from 2.2% to about 2.75%, from about 0.06% to about 0.1% carbon, about 14%, and preferably 16%, to about 20% cobalt, about 3% to 6% molybdenum, at least 0.001% and preferably at least

45 the deposited ash. The data given in Table IV illustrate that the excellent corrosion resistance characteristics of alloys within the invention are not detrimentally impaired in achieving the markedly improved stress-rupture properties. The corrosion tests were carried out by half immersion of the specimens tested (other half exposed to air) 50 in a molten mixture of sodium sulfate (75% by weight of the mixture) and sodium chloride (25% by weight) for sixteen hours at the various temperatures set forth in Table IV. The weight loss of the specimens was determined and is reported in Table IV. Alloy No. 18 (Alloy No. 8 of British Patent No. 959,509) devoid of both cobalt and molybdenum and containing 20% chromium, is included for purposes of comparison:

TABLE IV

| Alloy No. | Composition <sup>1</sup> (percent by weight) |      |      |      |       |      |       |       |       | Weight Loss, mg./cm. <sup>2</sup> After 16 hours |         |           |
|-----------|----------------------------------------------|------|------|------|-------|------|-------|-------|-------|--------------------------------------------------|---------|-----------|
|           | C                                            | Cr   | Ti   | Al   | Ti+Al | Co   | Mo    | Zr    | B     | 800° C.                                          | 900° C. | 1,000° C. |
| 18        | 0.07                                         | 20   | 2.5  | 1.2  | ----- | 0.05 | 0.003 | 613   | ----- | -----                                            | -----   | -----     |
| 6         | 0.068                                        | 31.0 | 1.90 | 0.55 | 18.0  | 4.68 | 0.06  | 0.004 | 4.3   | 4.1                                              | 6.9     | -----     |
| 13        | 0.043                                        | 29.4 | 1.43 | 0.56 | 19.7  | 3.98 | 0.05  | 0.003 | 2.4   | 5.1                                              | 6.2     | -----     |
| 15        | 0.09                                         | 30.9 | 2.14 | 0.65 | 18.0  | 4.48 | 0.06  | 0.003 | 2.4   | 5.1                                              | 6.9     | -----     |

<sup>1</sup> Alloys contained less than 0.3% silicon.

0.002% or 0.003% and up to about 0.006% boron, about 0.02% to 0.08% zirconium, with the balance being essentially nickel. Lower amounts of carbon, i.e., not more than 0.06%, can be suitably used particularly with aluminum contents of 0.7% to 1.1%.

Alloys of the present invention are suitable for use 70 as rotor blades and other stressed parts of gas turbines. The alloys are particularly useful in forming articles subjected in use to high stress and corrosive atmospheres at elevated temperatures, for example, parts of furnaces and air heaters. Apart from being used in the wrought form, the alloys can also be used for cast components.

It is important, as in the case of the alloys described in 75

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. A nickel-chromium-base alloy characterized by a high degree of corrosion resistance and stress-rupture characteristics at elevated temperatures, said alloy consisting essentially of about 27% to 35% chromium, about 1.5% to about 2.5% titanium, about 0.5% to about 1.1% aluminum, the total titanium plus aluminum being from about 2.2% to 2.75%, carbon at least 0.01% to about 0.1% with the proviso that the aluminum content is at least about 0.7% when the carbon content is in the range of 0.01% to 0.06%, about 14% to about 20% cobalt,

about 3% to 6% molybdenum, about 0.001% to 0.006% boron, about 0.02% to about 0.08% zirconium and the balance essentially nickel.

2. An alloy in accordance with claim 1 containing at least 0.7% aluminum, at least 0.06% carbon, and at least 16% cobalt.

#### References Cited

##### UNITED STATES PATENTS

|           |         |                 |        |
|-----------|---------|-----------------|--------|
| 3,177,075 | 4/1965  | Richards et al. | 75—171 |
| 3,207,599 | 9/1965  | Franklin et al. | 75—171 |
| 3,222,165 | 12/1965 | Bird et al.     | 75—171 |

##### FOREIGN PATENTS

|         |        |                |
|---------|--------|----------------|
| 959,509 | 6/1964 | Great Britain. |
|---------|--------|----------------|

RICHARD O. DEAN, *Primary Examiner.*

UNITED STATES PATENT OFFICE  
CERTIFICATE OF CORRECTION

Patent No. 3,408,179 Dated August 7, 1969

Inventor(s) HARRY LEWIS and RONALD ALFRED SMITH

It is certified that error appears in the above-identified patent and that said Letters Patent are hereby corrected as shown below:

Column 4, line 8, for "15" first occurrence, read --14--.

SIGNED AND  
SEALED

DEC 2 - 1969

(SEAL)

Attest:

Edward M. Fletcher, Jr.

Attesting Officer

WILLIAM E. SCHUYLER, JR.  
Commissioner of Patents